

## UNITED STATES PATENT OFFICE

1,954,333

WRAPPING PAPER FOR PHOTOGRAPHIC  
GOODS

Samuel E. Sheppard and Herbert J. Dietz,  
Rochester, N. Y., assignors to Eastman Kodak  
Company, Rochester, N. Y., a corporation of  
New York

No Drawing. Application May 13, 1930,  
Serial No. 452,127

8 Claims. (CL. 91—67.9)

This invention relates to a process and product  
for the wrapping of light-sensitive materials and  
particularly to the preparation of wrapping pa-  
pers having thereon various markings of con-  
trasting colors.

The paper which is usually employed for wrap-  
ping photographic plates and films is frequently  
the source of trouble in the sense that a fogging  
or desensitizing of the light-sensitive emulsions is  
10 effected. This is particularly liable to be the case  
in respect of roll film, as used in photographic  
roll film cameras, because of the various con-  
volutions of the film, one side being rolled up  
in contact with the emulsion, and the back of  
15 that wrapping paper coming in contact with the  
film support, or more usually, a gelatin coating  
on the back of said support. Any inequality of  
the paper, in regard to emanations or fogging  
vapors therefrom, is liable, therefore, by this im-  
20 mediate contact, to produce corresponding in-  
equalities of density on the developed film. This  
condition is liable to be accentuated by the pres-  
ence of imprints: signs, letters, or numerals, put  
upon the paper, as, for example to indicate the  
25 batch or roll number, the origin, or to signal to  
the operator the number of the particular ex-  
posure. Apart from mere mechanical offsetting,  
such imprints are liable to give pseudo-photo-  
graphic offsetting, whether by fogging (increase  
30 of local density on development) or by de-  
sensitizing (decrease of local density).

The inherent chemical emulsion fog of any  
photographic emulsion is liable to be enhanced or  
added to on storage or incubation in the presence  
35 of almost any organic material which is in any  
degree autoxidizable by reason of the produc-  
tion of peroxides, and especially the volatile hy-  
drogen peroxide. This is notably the case in cer-  
tain substances, such as drying oils, resins and  
40 the like. But even when such substances are re-  
duced to a minimum, it is extremely difficult,  
probably impossible to have organic materials  
present—and they are necessarily present, as the  
gelatin and the film support itself—without some  
45 degree of autoxidation taking place in the pres-  
ence of air and moisture. So that, although the  
fog due to this cause may be and is in good prac-  
tice reduced to a very small amount and in most  
instances to a slight veil not objectionable to the  
50 photographic use of such materials, yet a slight  
fog will normally be produced, and tend to in-  
crease somewhat with the age of the product, i. e.,  
with time of storage.

55 So long as this slight veil of fog is uniform  
over the plate, it is unobjectionable or harmless,  
but if anything occurs to locally interfere with  
the autoxidation of the paper (and of course its  
constituents) and consequently perceptibly en-  
60 hance or diminish this slight veil or fog, then this

differential reduces the utility of the product for  
photographic purposes.

An object of the present invention is to pro-  
vide a process for the preparation of materials  
which contact with light sensitive coatings, the 65  
former having no offsetting effect upon the coat-  
ings. By the term, offsetting effect, is meant the  
tendency of portions of light sensitive coatings  
to unevenly fog due to the stimulus of the sur-  
rounding materials. Another object of this in- 70  
vention is to provide a process for the prepara-  
tion of wrapping paper for photographic goods,  
such paper having no offsetting effect upon the  
coatings. Another object of this invention is to  
provide a process for the preparation of wrap- 75  
ping paper for photographic goods, such paper  
having no offsetting effect upon the photographic  
material wrapped therewith. Other objects will  
hereinafter appear.

We have found that if anyone of a number of 80  
substantially pure inorganic pigments and cer-  
tain lakes, (which, of course, consist of the com-  
pound resulting from the interaction of a mor-  
tard and a dye, the lake being preferably pre-  
pared in a state of fine subdivision), are sus- 85  
pended in a considerable quantity of gelatin or  
other colloid binder and dried, and are then  
brought into close contact with the sensitive sur-  
face of a photographic plate or film, which is  
then stored or incubated, that the area in contact 90  
with the pigmented or laked layer shows a ma-  
terially decreased or increased fog density be-  
cause the lake or pigment has an increased power  
of catalytically destroying hydrogen peroxide 95  
which is formed by autoxidation of the paper  
itself (or its constituents or even the binder used  
in the ink) and which peroxide, as known in the  
art, fogs a light sensitive emulsion. If the pig-  
mented or laked layer is held sufficiently far away 100  
from contact with the emulsion, no differen-  
tial impression is observable. Now it is evident  
that if such pigments be employed in making up  
an ink for impressing a photographic wrapping  
paper, which will frequently contain a black or 105  
red dye for producing opacity to light—the former  
generally being in direct contact with the film  
support or gelatin coating thereon and the latter,  
particularly when used in roll films, will be  
wound up in contact with the light-sensitive 110  
emulsion—that the uniform veiling action, part-  
ly due to the paper itself and partly due to the  
dye or pigment used in the paper will be locally  
reduced, so that undesirable off-setting effects  
will result on the developed film, and experi- 115  
ments show this to be the case.

We have found a method for the preparation of  
paper, cloth, organophilic cellulosic sheet or other  
wrapping materials for photographic or other  
light-sensitive goods whereby the disadvantages  
resulting from the use of dissimilar dyes may be 120

obviated. It consists as usual in loading the paper or coating thereon a pigment to make the paper opaque to light and, subsequent to this preliminary preparation, coating the paper with 5 a second pigment which may or may not have a contrasting color to the first pigment but which has substantially the same catalytic effect with regard to production or destruction of hydrogen peroxide as does the first pigment (namely that 10 in the paper) and, therefore, the same fogging or anti-fogging effect upon light-sensitive coatings as does the first pigment applied to the material. In some instances it has been found desirable to impregnate the paper while in the 15 formative stage with a size and a pigment, and subsequent to its fabrication in sheet form, printing thereon with a pigmented ink (to produce markings or identifications) which comprises as a binder the size used in first impregnation of the 20 paper. The pigment in both cases is, of course, of different colors, but their activity with regard to hydrogen peroxide and consequently their action on the photographic light-sensitive emulsion will be substantially the same, whether it be a 25 fogging or anti-fogging action upon the light-sensitive layer. In place of impregnating the fibers of the paper in its preliminary preparation, this sizing material may be applied to the surface thereof with equally good results.

30 The size which may be utilized for both the preliminary treatment of the paper as well as for the binder in the suspension of the second pigment may comprise any type of sizing or binding material which has, at the most, but slight action upon the light-sensitive emulsions. It is im- 35 material whether this slight activity be of the fogging or anti-fogging nature. The sizes which we have found useful have been engine size, such as purified rosin sizing plus starch, or tub sizing, e. g., animal size. Many other sizes having the 40 above qualities may be used, and such will come within the scope of this invention.

The pigments which we have found suitable 45 comprise a large number of both the organic and inorganic pigments, and in speaking of pigments in this application, we imply the broad dictionary meaning of that word, including all the coloring media. In selecting the pigment, whether it be for the preliminary treatment of the paper or the 50 subsequent treatment, it must be borne in mind that here again the activity of this pigment toward the light-sensitive coating should be relatively slight. It does not matter whether this activity be of the fogging or desensitizing nature. 55 It is advantageous, however, in order that the developed film or other sensitive surface be not deleteriously affected that the pigment has comparatively slight activity in this regard. We have found the following substantially pure pigments 60 give similar catalytic effect with regard to hydrogen peroxide and, therefore, the same anti-fogging effect under the specified conditions.

subsequently similar fogging action under like conditions:

| Name                                    | Chemical character                                                                                         |    |
|-----------------------------------------|------------------------------------------------------------------------------------------------------------|----|
| Fogging pigments:<br>Carbon blacks..... |                                                                                                            | 80 |
| Tuscan red.....                         |                                                                                                            |    |
| Fogging dyes:<br>Methylene blue.....    | Tetramethyl diamino-diphenaz-thionium chloride.                                                            |    |
| Victoria green.....                     | Zinc double chloride of para para tetramethyldiamino - tri - phenyl-carbinol anhydride.                    | 85 |
| Diazine black.....                      | Not listed.                                                                                                |    |
| Niagara blue.....                       | Sodium salt of diphenyl-diazo bis-S-amino - 1 - naphthol - 3:6 - disulphonic acid.                         |    |
| Pontamine fast black.....               | Sodium salt of 6 sulph-4-amino-a-naphthalene-azo-benzene-azo-3-sulpho-1-naphthol-7-azo-m-phenylenediamine. | 90 |
| Xylene blue.....                        | Sodium salt of disulphonic acid of m-hydroxy-tetra - ethyldiamino-tri-phenylcarbinol anhydride.            |    |
| National fast red S. conc.....          | Sodium salt of 4-sulpho-a-naphthalene-azo-p-naphthol.                                                      |    |
| Erie fast scarlet 8 B A.....            | Sodium salt of benzene-azo-7:7'disulpho-5:5'dihydroxy-naphthyl 2:2'urea-azo-p-acetylaminobenzene.          | 95 |
| Safranine G.....                        | Mixture of diamino-phenyl-ditolazonium chloride diamino-o-tolyl-ditolazonium chloride.                     |    |

100 In the preparing of papers or other materials, as described in our preferred process hereinabove disclosed, in some instances it may not be necessary to have a binder present in the pigment which is applied to the sized and pigmented paper, although this expedient will not in all cases give the optimum results as it is well known that papers will generally not hold as much pigment or dye when it contains little or no size. It is desirable that the pigments have 110 the same activity and likewise can be held in sufficient amounts by the paper while the amount of pigment of either type over a given area of the paper has substantially equal density. Should this process be employed, the size of the paper 115 should not harmfully act on the light-sensitive emulsions.

120 It will be evident from the above disclosure that we are not limited to any particular manner of preparing the paper or other material or applying thereto the sizing pigment or the contrasting pigments, the degree of color contrast desired governing the quantities of the dyes and the necessary size and binder used. Variations, therefore, in the quantity of these materials or in 125 similar pigments having equivalent activity, be it of the fogging or anti-fogging nature, will come within the scope of this invention and in no way sacrifice any of its advantages.

130 What we claim as our invention and desire to be secured by Letters Patent of the United States is:

1. Process for preparing papers which are intended for contact with light-sensitive materials which comprises loading the paper base with a 135 light excluding pigment and subsequently locally applying to the paper an ink in the form of identification marks, which ink comprises a contrasting pigment, both pigments having the same catalytic effect with regard to the hydrogen 140 peroxide produced by the autoxidation of materials comprised in the finished paper.

2. Process for preparing papers which are intended for contact with light-sensitive materials which comprises loading the paper with a 145 size and a light excluding pigment and subsequently locally applying to the paper an ink in the form of identification marks, which ink comprises a contrasting pigment and comprises, as a suspending medium, the same size as used in 150

|    | Name                                     | Chemical character       |
|----|------------------------------------------|--------------------------|
| 65 | Cobalt blue.....                         | Cobalt aluminum sulfate. |
|    | Chrome green.....                        | Chromium sesqui-oxide.   |
|    | Manganese oxide (brown).....             | Manganese di-oxide.      |
|    | Prussian blue.....                       | Ferric-ferrous-cyanide.  |
|    | Aquadag artificial graphite (black)..... | Graphitic carbon.        |
| 70 | Calcium alizarine lake (red brown).....  | Calcium alizarinate.     |

75 The following give substantially the same rate of autoxidation and production of hydrogen peroxide when associated with paper fibers and con-

the paper, both pigments having the same catalytic effect with regard to the hydrogen peroxide produced by the autoxidation of materials comprised in the finished paper.

5 3. Process for preparing papers which are intended for contact with light sensitive materials which comprises loading the paper base with a size and a light-excluding pigment and subsequently locally applying to the paper an ink in the form of identification marks, which ink comprises a contrasting pigment and a suspending medium therefor, the total catalytic effect of the size and pigment in the paper base with regard to the hydrogen peroxide produced 10 by the autoxidation of materials comprised in the finished paper being the same as the total catalytic effect, with regard to the hydrogen peroxide produced by the autoxidation of materials comprised in the finished paper, of the suspending medium and pigment comprised in 15 the ink.

4. A photographic wrapping paper intended for contact with light sensitive materials, comprising a paper base loaded with a light-excluding pigment and identification marks thereon composed of ink which comprises a contrasting pigment, both pigments having the same catalytic effect with regard to the hydrogen peroxide produced by the autoxidation of materials comprised in the finished paper.

5. A photographic wrapping paper intended for contact with light sensitive materials, comprising a paper base loaded with a size and a light-excluding pigment, and identification

marks thereon composed of ink which comprises a contrasting pigment and, as a suspending medium, the same size as is used in the paper, both pigments having the same catalytic effect with regard to the hydrogen peroxide produced by the autoxidation of materials comprised in the finished paper.

6. A photographic wrapping paper intended for contact with light-sensitive materials, comprising a paper baseloaded with a size and a light-excluding pigment, and identification marks thereon composed of ink which comprises a contrasting pigment and a suspending medium therefor, the total catalytic effect of the size and pigment in the paper base with regard to the hydrogen peroxide produced by the autoxidation of materials comprised in the finished paper being the same as the total catalytic effect, with regard to the hydrogen peroxide produced by the autoxidation of materials comprised in the finished paper, of the suspending medium and pigment comprised in the ink.

7. Process for the preparation of papers which contact with light-sensitive materials which comprises loading the paper with sizing and artificial graphite and subsequently applying thereto a color coating comprising sizing and manganese dioxide.

8. A photographic wrapping paper loaded with sizing and artificial graphite and marked with a color coating comprising sizing and manganese dioxide.

SAMUEL E. SHEPPARD.  
HERBERT J. DIETZ.

35

110

40

115

45

120

50

125

55

130

60

135

65

140

70

145

75

150

80

85

90

95